# EUROPEAN PATENT SPECIFICATION

(11) **EP 2 279 677 B1**
(45) Date of publication and mention of the grant of the patent: **28.10.2015**
(21) Application number: 09750521.8
(22) Date of filing: 15.05.2009
(51) Int. Cl.: A24B 15/28, A24D 1/00

(54) **MATERIAL CONTAINING FLAVORING AGENT FOR CIGARETTE, METHOD FOR PRODUCTION THEREOF, AND CIGARETTE**
AROMASTOFFHALTIGES MATERIAL FÜR EINE ZIGARETTE, HERSTELLUNGSVERFAHREN DAFÜR UND ZIGARETTE
MATIÈRE CONTENANT UN AGENT AROMATISANT POUR CIGARETTE, SON PROCÉDÉ DE PRODUCTION, ET CIGARETTE

(30) Priority: 19.05.2008 JP 2008131087
(43) Date of publication of application: 02.02.2011
(73) Proprietor: Japan Tobacco, Inc., Tokyo 105-8422 (JP)
(72) Inventor: TANAKA, Yasuo, TOKYO, 130-8603 (JP); KUSAKABE, Tatsuya, TOKYO, 130-8603 (JP); YAMAMOTO, Yuji, TOKYO, 130-8603 (JP)
(74) Representative: Isarpatent
(86) International application number: PCT/JP2009/059079
(87) International publication number: WO 2009/142159

(56) References cited:
- EP-A2- 0 464 324
- EP-A2- 0 908 109
- WO-A1-98/15191
- WO-A1-02/083827
- WO-A1-2009/021018
- WO-A2-2007/091181
- JP-A- 1 027 461
- JP-A- 1 027 461
- JP-A- 4 075 578
- JP-A- 9 028 366
- JP-A- 9 028 366
- JP-A- H11 509 566
- JP-A- 2007 023 065
- JP-B- 59 033 345
- JP-B2- 3 790 828
- US-A- 3 550 598

## Description

### Technical Field

The present invention relates to a process for producing a sheet-form flavor-containing material for a cigarette.

### Background Art

When menthol cigarettes are produced, a method of adding a flavor component such as menthol to cut tobacco in a solution state is adopted. This method has an advantage that by spraying or some other operation of the flavor solution, the flavor components can easily be added to the cut tobacco. However, when the addition amount of the flavor is increased in order to release a sufficient aroma at the time of smoking, the amount of a solvent is also increased. Therefore, at the time of the addition of the flavor solution, components containing a colorant and others are extracted from the cut tobacco with the solvent, so that a "stain" tends to be generated on the cigarette wrapper. Moreover, the flavor components, such as menthol, have volatility, so as to result in a drawback that the flavor components are dissipated when the cigarettes are stored over a long term, so that the flavor effect does not last. Furthermore, in the case of using a cigarette in which a charcoal filter is used to remove unpleasant taste in mainstream smoke of the cigarette, the flavors are adsorbed to the charcoal during a storage period, so that the flavors are significantly volatilized and dissipated, and thus, the cigarette also has a drawback that a decrease in the flavor effect becomes significant in storage.

Against this, techniques of encapsulating flavor components and adding the encapsulated components to a cigarette are reported in Japanese Patent No. 3790828 and Jpn. Pat. Appln. KOKAI Publication No. 4-75578. When such flavors are added to a cigarette, there is not caused a problem that the cigarette wrapper is stained as described above. Since the flavor components are encapsulated, the flavor components are restrained from being volatilized and dissipated when the cigarette is stored. However, in any one of the methods, a coating agent is gelled and brought into contact with the flavors to encapsulate the flavors. When the coating agent is gelled, the addition of a gelling agent, such as a metal chloride, is required. The addition of such a metal chloride causes a problem that, when the cigarette is combusted, a thermal decomposition product of the metal halide is entrained in the mainstream smoke. Furthermore, the method of Jpn. Pat. Appln. KOKAI Publication No. 4-75578 requires crashing the flavor-containing capsule when the cigarette is smoked.

JP 9028366 discloses a flavor-containing material for cigarette, wherein a flavor is coated with a gel of a polysaccharide which flavor-containing material is provided by: (i) mixing the polysaccharide with water and heating the mixture to prepare an aqueous solution of the polysaccharide; and (ii) adding the flavor and an emulsifier to the aqueous solution and kneading and emulsifying the solution and wherein the flavor is in a solid or a liquid and characterized in that is shaped into a sheet form.

JP 9028366 further discloses a process for producing a flavor-containing material for cigarette comprising steps of: (i) mixing a polysaccharide with water and heating the mixture to prepare an aqueous solution of the polysaccharide; and (ii) adding a flavor and an emulsifier to the aqueous solution of the polysaccharide and kneading and emulsifying the solution.

WO 98/1591 discloses a flavor-containing material for cigarette, wherein a flavor is coated with a gel of a polysaccharide which flavor-containing material is provided by: (i) mixing the polysaccharide with water and heating the mixture to prepare an aqueous solution of the polysaccharide; and (ii) adding the flavor and an emulsifier to the aqueous solution and kneading and emulsifying the solution (example 4), wherein the polysaccharide is a single component system of gellan gum and wherein the flavor is contained in 18 wt% or more, more preferably in 45 wt% or more and is in solid or liquid.

WO 98/1591 further discloses a process for producing a flavor-containing material for cigarette, comprising steps of: (i) mixing a polysaccharide with water and heating the mixture to prepare an aqueous solution of the polysaccharide; and (ii) adding a flavor and an emulsifier to the aqueous solution of the polysaccharide and kneading and emulsifying the solution (example 4).

US 3,550,598 discloses a flavor-containing material for a cigarette, wherein a flavor is coated with a gel of a polysaccharide. US 3,550,598 further discloses a flavor-containing material for cigarette wrapper wrapping the cut tobacco, wherein the flavor-containing material for cigarette is added to the cut tobacco wherein the sheet-form flavor-containing material for cigarette is shredded and added to the cut tobacco.

EP 0908109 discloses a flavor a flavor-containing material for cigarette, wherein the flavor is coated with a gel of a polysaccharide containing, which flavor-containing material is shaped into a sheet form.

EP 098109 also discloses a cigarette comprising a tobacco rod comprising cut tobacco and a cigarette wrapper wrapping the cut tobacco, wherein the sheet-form flavor-containing material is shredded and added to the cut tobacco (paragraph 10).

EP 0464324 discloses a flavoring granule for tobacco products, comprising a solid substrate granule of which comprises natural polysaccharides or derivatives thereof, and a flavor for tobacco products which is contained in said solid granule and is encapsulated in said solid granule so as to be released upon breakage of said solid granule, wherein said solid granule further contains casein as a diluent. Also disclosed is a preparation method thereof, by which the flavoring granule of large size and excellent sphere shape can be obtained.

JP 1027461 discloses a perfume in a solid or liquid state at room temperature which is mixed with a diluent such as a starch powder and calcium carbonate if necessary, and then, it is mixed with a solution of natural polysaccharide of its derivate such as alginate and carboxymethyl cellulose salt. The obtained mixture is preferably dropped and solidified in a hardening agent solution such as a metal salt of potassium or calcium. Or, a gel is produced from the mixture, and dropped and solidified in a solution of natural polysaccharide. Thus, such particles that the perfume is sealed in a solid particle comprising natural polysaccharide, or perfume particles coated with a coating film of natural polysaccharide are obtained.

WO 02/083827 discloses glucan capsules having a flavor component enclosed therein and obtained by spraying a heat-irreversibly coagulating glucan dispersion containing the flavor component into a gas stream at a temperature corresponding to the critical gelation point of glucan or higher to thereby enclose the flavor component followed by the coagulation/gelation of the glucan in this state to give capsules.

WO 2009/021018 discloses a flavor-containing material for cigarette, wherein a flavor is coated with a gel of a polysaccharide, the polysaccharide being a single component system of carrageenan, wherein the flavor is contained in 18 wt% or more, more preferably in 45 wt% or more and is in a solid or liquid.

WO 2009/021018 further discloses a flavor containing material being shaped into a sheet form and a cigarette comprising a tobacco rod comprising cut tobacco and a cigarette wrapper wrapping the cut tobacco, wherein the flavor-containing material for cigarette is shredded and added to the cut tobacco.

WO 2009/021018 further discloses a process for producing a flavor-containing material for cigarette, comprising steps of: (i) mixing a polysaccharide with water and heating the mixture to prepare an aqueous solution of the polysaccharide; and (ii) adding a flavor and an emulsifier to the aqueous solution of the polysaccharide and kneading and emulsifying the solution.

### Disclosure of Invention

An object of the present invention is to provide a process for producing a flavor-containing material for a cigarette in which a flavor is coated with a polysaccharide without adding any gelling agent, such as a metal chloride, to the material.

According to the present invention, there is provided a process for producing a sheet-form flavor-containing material for cigarette, characterized in that the process comprises steps of:
(i) mixing a polysaccharide with water and heating the mixture at a temperature of 60 to 90°C to prepare an aqueous solution of the polysaccharide;
(ii) adding a flavor and an emulsifier to the aqueous solution of the polysaccharide and kneading and emulsifying the solution to obtain an emulsified slurry; and
(iii) casting the emulsified slurry on a substrate and drying it to obtain a sheet form,
   wherein the polysaccharide is a single component system of tamarind gum, psyllium seed gum or konjak glucomannan, or a composition system of combined two or more components selected from the group consisting of tamarind gum, konjak glucomannan, cassia gum and psyllium seed gum.

### Brief Description of Drawings

FIG. 1 is a graph showing a flavor-retaining property when the storage of a cigarette is continued under normal environment conditions.
FIG. 2 is a graph showing a flavor-retaining property when the storage of a cigarette is continued under accelerated environment conditions.

### Best Mode for Carrying Out the Invention

The present invention will be described in more detail hereinafter.

The flavor-containing material used in the process for producing a sheet-form flavor-containing material for cigarette according to the invention is characterized in that a flavor is coated with a gel of a polysaccharide that contains no gelling agent.

As the flavor, various flavors may be used. For example, 1-menthol may be used.

The polysaccharide used in the invention can be gelled only by applying heat. Thus, no gelling agent is required. Accordingly, the flavor-containing material for cigarette according to the invention contains no gelling agent such as a metal chloride. Thus, for example, an unfavorable decomposed product of the chloride is not produced in the mainstream smoke during smoking.

In order to increase the flavor content of the flavor-containing material, it is necessary that the flavor is effectively coated with the polysaccharide. The present inventors have found that it is effective that a flavor and a polysaccharide are sufficiently kneaded and emulsified in a heated aqueous solution, and the emulsified state that the flavor coated with the gelled polysaccharide is present in the aqueous solution is maintained while the flavor-containing material is prepared. That is, in a flavor-containing material that can be sufficiently kneaded and emulsified and can keep the emulsified state, high flavor content can be finally obtained. On the other hand, it has been found that, in a system that cannot keep the emulsified state in the aqueous solution during the preparation of the material even when sufficient kneading and emulsifying are performed, high flavor content cannot be attained. The flavor-containing material of the invention may contain 18 wt% or more, preferably 60 wt% or more, more preferably 70 wt% or more of flavor.

The polysaccharide that can keep an emulsified state as described above is preferably a single component system of tamarind gum, psyllium seed gum or konjak glucomannan, or a composition system of combined two or more components selected from the group consisting of tamarind gum, konjak glucomannan, cassia gum and psyllium seed gum. At the time of the emulsification, it is preferred to use an ordinarily used emulsifier, such as lecithin, together.

By casting the flavor-containing material, prepared by kneading and emulsifying the flavor and the polysaccharide in an aqueous solution, on a substrate and drying, a sheet can be produced. This flavor-containing material sheet can be shredded and then added to cut tobacco.

The flavor-containing material can be kneaded and emulsified into a slurry state, which may be added to cut tobacco or a cigarette wrapper.

A cigarette to which the flavor-containing material produced according to the present invention is added has a higher flavor-retaining property than ordinary menthol cigarettes since the flavor is coated with the polysaccharide. For this reason, also when a charcoal filter is fitted thereto, the cigarette can have a flavor-retaining property without any problem.

The flavor-containing material for cigarette produced according to the invention is prepared by a process comprising steps of:
(i) mixing a polysaccharide with water and heating the mixture at a temperature of 60 to 90°C to prepare an aqueous solution of the polysaccharide;
(ii) adding a flavor and an emulsifier to the aqueous solution of the polysaccharide and kneading and emulsifying the solution to obtain an emulsified slurry; and
(iii) casting the emulsified slurry on a substrate and drying it to obtain a sheet form,
   wherein the polysaccharide is a single component system of tamarind gum, psyllium seed gum or konjak glucomannan, or a composition system of combined two or more components selected from the group consisting of tamarind gum, konjak glucomannan, cassia gum and psyllium seed gum.

In the step (i), a polysaccharide and water is mixed with each other and then the mixture is once heated, whereby the polysaccharide is imparted a property capable of gelling in standing to cool. The heating temperature is preferably a temperature of 60 to 90°C. Effects of the heating include followings: the solubility of the gelled polysaccharide in water is improved; further, the polysaccharide is imparted a property capable of gelling in standing to cool; the flavor added in the step (ii) is made into a melted state and, at the same time, the viscosity of the aqueous solution of the polysaccharide is lowered, thereby facilitating the emulsification thereof with the flavor; further, it is found that, when the heated aqueous solution of the polysaccharide is kneaded and emulsified with the flavor in the step (ii), the emulsified state can be kept during preparation of the flavor-containing material.

Next, in the step (ii), a flavor and an emulsifier are added to the aqueous solution of the polysaccharide, and the mixture is kneaded and emulsified. Various types of flavor may be used as described above, and 1-menthol, for example, may be used. The flavor is taken in the aqueous solution of the polysaccharide from the step (i) by kneading and is present in an emulsified state. As described above, this emulsified state is kept during preparation of the flavor-containing material, which makes it possible to prepare a flavor-containing material of high flavor content. In other words, a smoking article containing this flavor-containing material can produce a more aroma during smoking. The flavor content of the flavor-containing material is preferably 18% or more, more preferably 60% or more, in particular preferably 70% or more.

### EXAMPLES

Hereinafter, the invention will be described in more detail by way of examples.

### Preparation of a flavor-containing material for cigarette according to the invention

A flavor-containing material for cigarette of the invention is prepared by use of a polysaccharide described below as a coating agent. The polysaccharides include tamarind gum, which is extracted from seed resin and has a structure of xyloglucan, psyllium seed gum, which is extracted from seed resin and is an acidic polysaccharide having a structure having a main chain of xylan and side chains of arabinose or the like, konjak glucomannan, which is extracted from tuberous roots of konjak, and any starch (which may be various raw materials thereof or soluble starch). Of them, tamarind gum, psyllium seed gum, or konjak glucomannan may be used as a single component system. The polysaccharide used in the present invention may be a composition system of combined two or more components selected from the group consisting of the polysaccharides tamarind gum, psyllium seed gum, cassia gum and konjak glucomannan. The process for preparing the flavor-containing material for cigarette of the present invention is as follows. First, while a polysaccharide (single component system or composition system) is heated, the polysaccharide is dissolved in water. To this aqueous solution at the heating temperature of 60 to 90°C , a flavor in a liquid state (or melted state) and an emulsifier are added, and then the liquid is kneaded and emulsified. Subsequently, in the state that this emulsified state is kept, the emulsion is cast and then the water in which the polysaccharide is dissolved is evaporated to form a sheet of the objective flavor-containing material for cigarette. With respect to a flavor-containing material for cigarette prepared using various types of polysaccharides, and a flavor delivery in cigarette smoke in a case where the material is added to a cigarette, actually examined results are described below as examples. The intended selection of flavors, types of an emulsifier, and others are mere examples.

### Reference Examples 1 to 13 and 17 to 19

κ-Carrageenan (CARRAGEENAN CS-530, San-Ei Gen F.F.I., Inc.), which is extracted from red algae seaweed was selected as a single polysaccharide and 1-menthol (special grade, Wako Pure Chemical Industries, Ltd.) was selected as a flavor, respectively. A flavor-containing material for cigarette of Ref. Example 1 was prepared by the following procedures.

To 5 g of K-carrageenan added was 100 mL of water, which was heated in a thermostat bath of 80°C to dissolve K-carrageenan sufficiently in water. Added thereto were 25 g of l-menthol and 2 mL of a 5% aqueous solution of lecithin (Sunlecithin A-1, Taiyo Kagaku Co., Ltd.), which was sufficiently emulsified by means of a homogenizer (high performance mixer DMM, ATEC Japan Co., Ltd.). This emulsified slurry was cast on a substrate into a sheet form, which was dried in a forced air circulation dryer of 40°C for one week (the thickness of the dried film: 0.1 mm). At this time, the emulsified state of the mixture was kept until the flavor-containing material was dried.

The prepared sheet-form flavor-containing material for cigarette of Ref. Example 1 contained about 80 wt% of menthol. Thus, a satisfactory amount of menthol could be added.

The flavor-containing material of the present invention also has a function of suppressing the volatility of the flavor. For example, the flavor-containing material for cigarette of Ref. Example 1 was continued to be stored under accelerated environment conditions (cyclic environments between a condition of 50°C and 60% humidity for 14 hours and a condition of 30°C and 70% humidity for 10 hours imitating the inside of a stock space of an automatic vending machine in summer). Also in this case, the flavor-containing material contained 73.5 wt% of menthol in the total weight of the material after one week, and 73.0 wt% after one month. From the results, it is found that the cigarette in which the flavor-containing material for cigarette according to the invention is added has a very high flavor-retaining property compared to any ordinary menthol cigarette having cut tobacco added with menthol, when the cigarette is stored over a long term or in a stock space of an automatic vending machine in summer and when a charcoal filter is fitted to the cigarette in order to remove unpleasant taste in the cigarette mainstream smoke.

Cigarettes were tested for menthol delivery. First, cigarette samples of Ref. Examples 2 and 3 fitted with a plain filter for which a tar value was designed to about 10 mg. Here, the cigarettes of Ref. Example 2 had cut tobacco added with 3% of the flavor-containing material for cigarette of Ref. Example 1, and the cigarettes of Ref. Example 3 had cut tobacco added with 5% of the flavor-containing material for cigarette of Ref. Example 1. At this time, in each of Ref.Examples 2 and 3, the flavor-containing material for cigarette of Ref. Example 1 could be added without causing the problem of a stain on the wrapper. The occurrence of a stain on the wrapper was observed visually. The cigarette of Ref. Example 2 provided a menthol delivery of 0.91 mg per cigarette (with a ratio of menthol to tar of 0.086), and the cigarette of Ref. Example 3 provided a menthol delivery of 2.09 mg per cigarette (with a ratio of menthol to tar of 0.186). These were sufficient deliveries for menthol cigarettes.

Also, cigarettes of Ref. Example 2 fitted with a charcoal filter were produced. Specifically, the cigarettes of Ref. Example 2 were fitted with a charcoal filter (a charcoal amount of 40 mg/filter), and the cigarettes were evaluated for the flavor-retaining property when the cigarettes were stored under ordinary environment conditions (22°C, and a humidity of 60%) and under accelerated environment conditions (as described above). FIG. 1 shows the results under the ordinary environment conditions, FIG. 2 shows the results under the accelerated environment conditions. The horizontal axis in FIG. 1 shows the elapsed days under the ordinary environment conditions, and that in FIG. 2 shows the elapsed days under the accelerated environment conditions. In each of FIGS. 1 and 2, the vertical axis shows the amount of menthol in smoke. In each of FIGS. 1 and 2, circular marks show the results for the cigarettes of Ref. Example 2, and triangular marks show those for the cigarettes of Comparative Example 1 described below.

### Comparative Example 1

Cigarettes equivalent to the current menthol products were produced. The menthol was added to cut tobacco by use of a solvent. In the same manner as in Ref. Example 2, the cigarettes were continued to be stored under ordinary environment conditions (22°C, and a humidity of 60%) and accelerated environment conditions (the above-mentioned environment imitating inside of a stock space of an automatic vending machine in summer), and then the flavor-retaining property was evaluated. The results are also shown in FIGS. 1 and 2.

From the measured results of the flavor-retaining property during a period of time in storage, it was clearly found the followings. The cigarettes of Ref. Example 2 had smaller reduction in the menthol amount in the smoke even when the elapsed days in storage increased, compared with the cigarettes of Comparative Example 1, to which menthol was added by use of the solvent in accordance with the production of the current products. This situation appeared as a remarkable difference, in particular, when the cigarettes were stored under the accelerated environment conditions imitating an automatic vending machine in summer shown in FIG. 2. Specifically, the cigarettes of Comparative Example 1, to which menthol was added by use of the solvent in accordance with the production of the current products, provided a menthol delivery of 0.571 mg per cigarette (with a ratio of menthol to tar of 0062) before the storage. The cigarette samples stored in the form of a 20-cigarette package for three months under the ordinary environment conditions (temperature: 22°C, and humidity: 60%) provided a menthol delivery of 0.162 mg per cigarette (with a ratio of menthol to tar of 0.018), which was reduced to about 1/3 of that before the storage. By contrast, the cigarettes of Ref. Example 2 provided a menthol delivery of 0.803 mg per cigarette (with a ratio of menthol to tar of 0.084) before the storage. The cigarette samples stored in the form of a 20-cigarette package same as above for three months under the ordinary environment conditions provided a sufficient menthol delivery of 0.676 mg per cigarette (with a ratio of menthol to tar of 0.070). Thus, it was found that about 84% of the initial value before the storage was retained.

The cigarettes of Comparative Example 1 stored in the form of a 20-cigarette package for three months under the accelerated environment conditions, imitating an automatic vending machine in summer, provided a menthol delivery of 0.043 mg per cigarette (with a ratio of menthol to tar of 0.005), which was reduced to about 1/10 of that before the storage. By contrast, the cigarettes of Ref. Example 2 after the same elapsed period of storage provided a sufficient menthol delivery of 0.626 mg per cigarette (with a ratio of menthol to tar of 0.065). Thus, about 78% of the initial value before the storage could be retained.

From these results, it is confirmed that, when the flavor-containing material according to the invention is used to add a flavor component such as menthol to cigarettes, there are provided cigarettes which can exhibit a sufficient flavor amount (i.e., a sufficient flavor delivery) and a sufficient flavor-retaining property during storage.

### Ref. Example 4

A composition system of κ-carrageenan and locust bean gum (Bistop D-2050, San-Ei Gen F.F.I., Inc.), which is a galactomannan extracted from tree seeds, mixed at a weight ratio of 8:2 was selected as a polysaccharide, and l-menthol was selected as a flavor. A flavor-containing material for cigarette was prepared by the following procedures.

To 4 g of κ-carrageenan and 1 g of locust bean gum added was 100 mL of water, which was heated in a thermostat bath of 80°C to dissolve the polysaccharides sufficiently in water. Added thereto were 25 g of l-menthol and 2 mL of a 5% aqueous solution of lecithin as an emulsifier, which was sufficiently emulsified by means of a homogenizer. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 76 wt% of menthol. Thus, a satisfactory amount of menthol could be added.

The flavor-containing material for cigarette of Ref. Example 4 was blended in 5% by weight ratio to cut tobacco, and a cigarette with a tar value designed to about 10 mg was produced. At this time, the flavor-containing material for cigarette of Ref. Example 4 could be added without causing the problem of a stain on the wrapper. Further, the cigarette was fitted with a plain filter. The cigarette provided a menthol delivery of 1.82 mg per cigarette (with a ratio of menthol to tar of 0.170). This was a sufficient delivery for a menthol cigarette.

### Ref. Example 5

A composition system of K-carrageenan and guar gum (Bistop D-2029, San-Ei Gen F.F.I., Inc.), which is a galactomannan extracted from tree seeds, mixed at a weight ratio of 8:2 was selected as a polysaccharide material, and l-menthol was selected as a flavor. A flavor-containing material for cigarette was prepared by the following procedures.

To 4 g of κ-carrageenan and 1 g of guar gum added was 100 mL of water, which was heated in a thermostat bath of 80°C to dissolve the polysaccharides sufficiently in water. Added thereto were 25 g of 1-menthol and 2 mL of a 5% aqueous solution of lecithin as an emulsifier, which was sufficiently emulsified by means of a homogenizer. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 84 wt% of menthol. Thus, a satisfactory amount of menthol could be added.

The flavor-containing material for cigarette of Ref. Example 5 was blended in 5% by weight ratio to cut tobacco, and a cigarette with a tar value designed to about 10 mg was produced. At this time, the flavor-containing material for cigarette of Ref. Example 5 could be added without causing the problem of a stain on the wrapper. Further, the cigarette was fitted with a plain filter. The cigarette provided a menthol delivery of 1.80 mg per cigarette (with a ratio of menthol to tar of 0.173). This was a sufficient delivery for a menthol cigarette.

### Ref. Example 6

Agar (special grade, Wako Pure Chemical Industries, Ltd.), which is extracted from red algae seaweed, was selected as a single polysaccharide and 1-menthol was selected as a flavor. A flavor-containing material for cigarette was prepared by the following procedures.

To 5 g of powdery agar added was 100 mL of water, which was heated in a thermostat bath of 80°C to dissolve agar sufficiently in water. Added thereto were 25 g of l-menthol and 2 mL of a 5% aqueous solution of lecithin as an emulsifier, which was sufficiently emulsified by means of a homogenizer. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 90 wt% of menthol. Thus, a satisfactory amount of menthol could be added.

The flavor-containing material for cigarette of Ref. Example 6 was blended in 5% by weight ratio to cut tobacco, and a cigarette with a tar value designed to about 10 mg was produced. At this time, the flavor-containing material for cigarette of Ref. Example 6 could be added without causing the problem of a stain on the wrapper. Further, the cigarette was fitted with a plain filter. The cigarette provided a menthol delivery of 2.15 mg per cigarette (with a ratio of menthol to tar of 0.201). This was a sufficient delivery for a menthol cigarette.

### Ref. Example 7

A composition system of gellan gum (Kelco gel, America CP Kelco), which is a polysaccharide produced by the metabolism of microorganisms, and tamarind gum (Bistop D-2032, San-Ei Gen F.F.I., Inc.), which is extracted from tree seeds and has a xyloglucan structure, mixed at a weight ratio of 1:1 was selected as a polysaccharide, and l-menthol was selected as a flavor. A flavor-containing material for cigarette was prepared by the following procedures.

To 1.0 g of gellan gum and 1.0 g of tamarind gum added was 100 mL of water, which was heated in a thermostat bath of 80°C to dissolve the polysaccharides sufficiently in water. Added thereto were 10 g of 1-menthol and 1.6 mL of a 5% aqueous solution of lecithin as an emulsifier, which was sufficiently emulsified by means of a homogenizer. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 85 wt% of menthol. Thus, a satisfactory amount of menthol could be added.

The flavor-containing material for cigarette of Ref. Example 7 was blended in 5% by weight ratio to cut tobacco, and a cigarette with a tar value designed to about 10 mg was produced. At this time, the flavor-containing material for cigarette of Ref. Example 7 could be added without causing the problem of a stain on the wrapper. Further, the cigarette was fitted with a plain filter. The cigarette provided a menthol delivery of 2.40 mg per cigarette (with a ratio of menthol to tar of 0.209). This was a sufficient delivery for a menthol cigarette.

### Ref. Example 8

A composition system of xanthan gum (SAN ACE NXG-S, San-Ei Gen F.F.I., Inc.), which is a polysaccharide produced by the metabolism of microorganisms, and locust bean gum mixed at a weight ratio of 1:1 was selected as a polysaccharide, and l-menthol was selected as a flavor. A flavor-containing material for cigarette was prepared by the following procedures.

To 1.5 g of xanthan gum and 1.5 g of locust bean gum added was 100 mL of water, which was heated in a thermostat bath of 80°C to dissolve the polysaccharides sufficiently in water. Added thereto were 15 g of 1-menthol and 1.2 mL of a 5% aqueous solution of lecithin as an emulsifier, which was sufficiently emulsified by means of a homogenizer. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 65 wt% of menthol. Thus, a satisfactory amount of menthol could be added.

The flavor-containing material for cigarette of Ref. Example 8 was blended in 5% by weight ratio to cut tobacco, and a cigarette with a tar value designed to about 10 mg was produced. At this time, the flavor-containing material for cigarette of Ref. Example 8 could be added without causing the problem of a stain on the wrapper. Further, the cigarette was fitted with a plain filter. The cigarette provided a menthol delivery of 2.25 mg per cigarette (with a ratio of menthol to tar of 0.184). This was a sufficient delivery for a menthol cigarette.

### Ref. Example 9

A composition system of xanthan gum and tara gum (Bistop D-2101, San-Ei Gen F.F.I., Inc.), which is a galactomannan extracted from tree seeds, mixed at a weight ratio of 1:1 was selected as a polysaccharide, and l-menthol was selected as a flavor. A flavor-containing material for cigarette was prepared by the following procedures.

To 1.5 g of xanthan gum and 1.5 g of tara gum added was 100 mL of water, which was heated in a thermostat bath of 80°C to dissolve the polysaccharides sufficiently in water. Added thereto were 15 g of 1-menthol and 1.2 mL of a 5% aqueous solution of lecithin as an emulsifier, which was sufficiently emulsified by means of a homogenizer. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 77 wt% of menthol. Thus, a satisfactory amount of menthol could be added.

The flavor-containing material for cigarette of Ref. Example 9 was blended in 5% by weight ratio to cut tobacco, and a cigarette with a tar value designed to about 10 mg was produced. At this time, the flavor-containing material for cigarette of Ref. Example 9 could be added without causing the problem of a stain on the wrapper. Further, the cigarette was fitted with a plain filter. The cigarette provided a menthol delivery of 2.09 mg per cigarette (with a ratio of menthol to tar of 0.191). This was a sufficient delivery for a menthol cigarette.

### Ref. Example 10

A composition system of xanthan gum and konjak glucomannan (fine konjak powder, Konjak Material Commerce and Industry Co-Operative Association of Gunma Prefecture in Japan), which is extracted from tuberous roots of konjak, mixed at a weight ratio of 1:1 was selected as a polysaccharide, and l-menthol was selected as a flavor. A flavor-containing material for cigarette was prepared by the following procedures.

To 1.5 g of xanthan gum and 1.5 g of konjak glucomannan added was 100 mL of water, which was heated in a thermostat bath of 80°C to dissolve the polysaccharides sufficiently in water. Added thereto were 15 g of l-menthol and 1.2 mL of a 5% aqueous solution of lecithin as an emulsifier, which was sufficiently emulsified by stirring with hand. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 76 wt% of menthol. Thus, a satisfactory amount of menthol could be added.

The flavor-containing material for cigarette of Ref. Example 10 was blended in 5% by weight ratio to cut tobacco, and a cigarette with a tar value designed to about 10 mg was produced. At this time, the flavor-containing material for cigarette of Ref. Example 10 could be added without causing the problem of a stain on the wrapper. Further, the cigarette was fitted with a plain filter. The cigarette provided a menthol delivery of 2.10 mg per cigarette (with a ratio of menthol to tar of 0.184). This was a sufficient delivery for a menthol cigarette.

### Ref. Example 11

A composition system of xanthan gum and tamarind gum mixed at a weight ratio of 1:1 was selected as a polysaccharide, and l-menthol was selected as a flavor. A flavor-containing material for cigarette was prepared by the following procedures.

To 1.5 g of xanthan gum and 1.5 g of tamarind gum added was 100 mL of water, which was heated in a thermostat bath of 80°C to dissolve the polysaccharides sufficiently in water. Added thereto were 15 g of 1-menthol and 1.2 mL of a 5% aqueous solution of lecithin as an emulsifier, which was sufficiently emulsified by stirring with hand. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 67 wt% of menthol. Thus, a satisfactory amount of menthol could be added.

The flavor-containing material for cigarette of Ref. Example 11 was blended in 5% by weight ratio to cut tobacco, and a cigarette with a tar value designed to about 10 mg was produced. At this time, the flavor-containing material for cigarette of Ref. Example 11 could be added without causing the problem of a stain on the wrapper. Further, the cigarette was fitted with a plain filter. The cigarette provided a menthol delivery of 1.23 mg per cigarette (with a ratio of menthol to tar of 0.140). This was a sufficient delivery for a menthol cigarette.

### Ref. Example 12

A composition system of xanthan gum and starch (reagent originating from corn, Wako Pure Chemical Industries, Ltd.) mixed at a weight ratio of 1:1 was selected as a polysaccharide, and l-menthol was selected as a flavor. A flavor-containing material for cigarette was prepared by the following procedures.

To 2.0 g of xanthan gum and 2.0 g of starch added was 100 mL of water, which was heated in a thermostat bath of 80°C to dissolve the polysaccharides sufficiently in water. Added thereto were 20 g of 1-menthol and 1.6 mL of a 5% aqueous solution of lecithin as an emulsifier, which was sufficiently emulsified by stirring with hand. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 50 wt% of menthol. Thus, a satisfactory amount of menthol could be added.

The flavor-containing material for cigarette of Ref. Example 12 was blended in 10% by weight ratio to cut tobacco, and a cigarette with a tar value designed to about 10 mg was produced. At this time, the flavor-containing material for cigarette of Example 12 could be added without causing the problem of a stain on the wrapper. Further, the cigarette was fitted with a plain filter. The cigarette provided a menthol delivery of 1.93 mg per cigarette (with a ratio of menthol to tar of 0.183). This was a sufficient delivery for a menthol cigarette.

### Ref. Example 13

A composition system of locust bean gum and a starch (reagent originating from corn, Wako Pure Chemical Industries, Ltd.) mixed at a weight ratio of 1:1; and a composition system of locust bean gum and a starch (soluble reagent, Wako Pure Chemical Industries, Ltd.) mixed at a weight ratio of 1:1 were selected as polysaccharides, and l-menthol was selected as a flavor. A flavor-containing material for cigarette was prepared by the following procedures.

To 2.5 g of locust bean gum and 2.5 g of each of the starches added was 100 mL of water, which was heated in a thermostat bath of 80°C to dissolve the polysaccharides sufficiently in water. Added thereto were 25 g of l-menthol and 2 mL of a 5% aqueous solution of lecithin as an emulsifier, which was sufficiently emulsified by means of a homogenizer. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 65 wt% of menthol in the case of using the starch originating from corn, and was measured to contain about 25 wt% of menthol in the case of using the soluble starch. Thus, a satisfactory amount of menthol could be added.

Each of the flavor-containing materials for cigarette of Ref. Example 13 was blended in about 10% by weight ratio to cut tobacco in the case of using the starch originating from corn and in about 20% by weight ratio to cut tobacco in the case of using the soluble starch, and cigarettes with a tar value designed to about 10 mg were produced. At this time, each of the flavor-containing materials for cigarette of Ref. Example 13 could be added without causing the problem of a stain on the wrapper. Further, each of the cigarettes was fitted with a plain filter.

The cigarette using the starch originating from corn provided a menthol delivery of 2.59 mg per cigarette (with a ratio of menthol to tar of 0.209). The cigarette using the soluble starch provided a menthol delivery of 2.30 mg per cigarette (with a ratio of menthol to tar of 0.216). These were sufficient deliveries for menthol cigarettes.

### Example 14

Konjak glucomannan was selected as a single polysaccharide and l-menthol was selected as a flavor. A flavor-containing material for cigarette was prepared by the following procedures.

To 100 mL of water, while heated in a thermostat bath of 80°C, added were 25 g of l-menthol and 2 mL of a 5% aqueous solution of lecithin as an emulsifier for sufficient dissolving, which was sufficiently emulsified by means of a homogenizer. Added thereto was 5 g of konjak glucomannan while dissolving, which was further kneaded and emulsified. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 20 wt% of menthol. Thus, a satisfactory amount of menthol could be added.

The flavor-containing material for cigarette of Example 14 was blended in 20% by weight ratio to cut tobacco, and a cigarette with a tar value designed to about 10 mg was produced. At this time, the flavor-containing material for cigarette of Example 14 could be added without causing the problem of a stain on the wrapper. Further, the cigarette was fitted with a plain filter. The cigarette provided a menthol delivery of 2.05 mg per cigarette (with a ratio of menthol to tar of 0.203). This was a sufficient delivery for a menthol cigarette.

### Example 15

Tamarind gum was selected as a single polysaccharide and l-menthol was selected as a flavor. A flavor-containing material for cigarette was prepared by the following procedures.

To 3 g of tamarind gum added was 100 mL of water, which was heated in a thermostat bath of 80°C to dissolve tamarind gum sufficiently in water. Added thereto were 15 g of l-menthol and 1.2 mL of a 5% aqueous solution of lecithin as an emulsifier, which was sufficiently emulsified by means of a homogenizer. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 18 wt% of menthol. Thus, a satisfactory amount of menthol could be added.

The flavor-containing material for cigarette of Example 15 was blended in 20% by weight ratio to cut tobacco, and a cigarette with a tar value designed to about 10 mg was produced. At this time, the flavor-containing material for cigarette of Example 15 could be added without causing the problem of a stain on the wrapper. Further, the cigarette was fitted with a plain filter. The cigarette provided a menthol delivery of 0.71 mg per cigarette (with a ratio of menthol to tar of 0.064). This was a sufficient delivery for a menthol cigarette.

### Example 16

Tamarind gum was selected as a single polysaccharide and l-menthol was selected as a flavor. A flavor-containing material for cigarette was prepared by the following procedures.

To 2 g of tamarind gum added was 100 mL of water, which was heated in a thermostat bath of 80°C to dissolve tamarind gum sufficiently in water. Added thereto were 20 g of l-menthol and 1.2 mL of a 5% aqueous solution of lecithin as an emulsifier, which was sufficiently emulsified by means of a homogenizer. Added thereto was 40 mL of ethyl alcohol (special grade, Wako Pure Chemical Industries, Ltd.), which was emulsified further sufficiently by means of a homogenizer. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 71 wt% of menthol. Thus, a satisfactory amount of menthol could be added.

The flavor-containing material for cigarette of Example 16 was blended in 5% by weight ratio to cut tobacco, and a cigarette with a tar value designed to about 10 mg was produced. At this time, the flavor-containing material for cigarette of Example 16 could be added without causing the problem of a stain on the wrapper. Further, the cigarette was fitted with a plain filter. The cigarette provided a menthol delivery of 2.20 mg per cigarette (with a ratio of menthol to tar of 0.187). This was a sufficient delivery for a menthol cigarette.

### Ref. Example 17

Gellan gum was selected as a single polysaccharide and l-menthol was selected as a flavor. A flavor-containing material for cigarette was prepared by the following procedures.

To 2 g of gellan gum added was 100 mL of water, which was heated in a thermostat bath of 80°C to dissolve gellan gum sufficiently in water. Added thereto were 10 g of l-menthol and 1.6 mL of a 5% aqueous solution of lecithin as an emulsifier, which was sufficiently emulsified by means of a homogenizer. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 80 wt% of menthol. Thus, a satisfactory amount of menthol could be added.

The flavor-containing material for cigarette of Ref. Example 17 was blended in 5% by weight ratio to cut tobacco, and a cigarette with a tar value designed to about 10 mg was produced. At this time, the flavor-containing material for cigarette of Ref. Example 17 could be added without causing the problem of a stain on the wrapper. Further, the cigarette was fitted with a plain filter. The cigarette provided a menthol delivery of 2.27 mg per cigarette (with a ratio of menthol to tar of 0.180). This was a sufficient delivery for a menthol cigarette.

### Ref. Example 18

A composition system of cassia gum (RheoRanger SR, Noveon, Inc. in USA), which is a galactomannan extracted from tree seeds, and K-carrageenan mixed at a weight ratio of 1:1 was selected as a polysaccharide, and l-menthol was selected as a flavor. A flavor-containing material for cigarette was prepared by the following procedures.

To 1.5 g of cassia gum and 1.5 g of K-carrageenan added was 100 mL of water, which was heated in a thermostat bath of 80°C to dissolve the polysaccharides sufficiently in water. Added thereto were 15 g of 1-menthol and 1.2 mL of a 5% aqueous solution of lecithin as an emulsifier, which was sufficiently emulsified by means of a homogenizer. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 77 wt% of menthol. Thus, a satisfactory amount of menthol could be added.

The flavor-containing material for cigarette of Ref. Example 18 was blended in 5% by weight ratio to cut tobacco, and a cigarette with a tar value designed to about 10 mg was produced. At this time, the flavor-containing material for cigarette of Ref. Example 18 could be added without causing the problem of a stain on the wrapper. Further, the cigarette was fitted with a plain filter. The cigarette provided a menthol delivery of 0.94 mg per cigarette (with a ratio of menthol to tar of 0.094). This was a sufficient delivery for a menthol cigarette.

### Ref. Example 19

A composition system of cassia gum and xanthan gum mixed at a weight ratio of 7:3 was selected as a polysaccharide, and l-menthol was selected as a flavor. A flavor-containing material for cigarette was prepared by the following procedures.

To 2.1 g of cassia gum and 0.9 g of xanthan gum added was 100 mL of water, which was heated in a thermostat bath of 80°C to dissolve the polysaccharides sufficiently in water. Added thereto were 15 g of 1-menthol and 1.2 mL of a 5% aqueous solution of lecithin as an emulsifier, which was sufficiently emulsified by means of a homogenizer. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 77 wt% of menthol. Thus, a satisfactory amount of menthol could be added.

The flavor-containing material for cigarette of Ref. Example 19 was blended in 5% by weight ratio to cut tobacco, and a cigarette with a tar value designed to about 10 mg was produced. At this time, the flavor-containing material for cigarette of Ref. Example 19 could be added without causing the problem of a stain on the wrapper. Further, the cigarette was fitted with a plain filter. The cigarette provided a menthol delivery of 0.49 mg per cigarette (with a ratio of menthol to tar of 0.051). This was a sufficient delivery for a menthol cigarette.

### Example 20

Psyllium seed gum (PG 200, MRC Polysaccharide Co., Ltd.), which is extracted from tree seeds and is an acidic polysaccharide having a structure with a main chain of xylan and side chains of arabinose was selected as a single polysaccharide and l-menthol was selected as a flavor. A flavor-containing material for cigarette was prepared by the following procedures.

To 4 g of psyllium seed gum added was 100 mL of water, which was heated in a thermostat bath of 80°C to dissolve the polysaccharide sufficiently in water. Added thereto were 20 g of l-menthol and 1.6 mL of a 5% aqueous solution of lecithin as an emulsifier, which was sufficiently emulsified by means of a homogenizer. This emulsified slurry was cast on a substrate into a sheet form, which was dried in a forced air circulation dryer of 40°C for one week. At this time, the emulsified state of the mixture was kept until the flavor-containing material was dried.

The prepared sheet-form flavor-containing material for cigarette was measured to contain about 73 wt% of menthol. Thus, a satisfactory amount of menthol could be added.

The flavor-containing material for cigarette of Example 20 was blended in 5% by weight ratio to cut tobacco, and a cigarette with a tar value designed to about 10 mg was produced. At this time, the flavor-containing material for cigarette of Example 20 could be added without causing the problem of a stain on the wrapper. Further, the cigarette was fitted with a plain filter. The cigarette provided a menthol delivery of 0.66 mg per cigarette (with a ratio of menthol to tar of 0.066). This was a sufficient delivery for a menthol cigarette.

## Claims

1. A process for producing a sheet-form flavor-containing material for cigarette, **characterized in that** the process comprises steps of:
(i) mixing a polysaccharide with water and heating the mixture at a temperature of 60 to 90°C to prepare an aqueous solution of the polysaccharide;
(ii) adding a flavor and an emulsifier to the aqueous solution of the polysaccharide and kneading and emulsifying the solution to obtain an emulsified slurry; and
(iii) casting the emulsified slurry on a substrate and drying it to obtain a sheet form, wherein the polysaccharide is a single component system of tamarind gum, psyllium seed gum or konjak glucomannan, or a composition system of combined two or more components selected from the group consisting of tamarind gum, konjak glucomannan, cassia gum and psyllium seed gum.

2. The process according to claim 1, **characterized in that** the process further comprises the step of shredding the obtained sheet-form flavor-containing material for cigarette.

3. The process according to claim 1 or 2, **characterized in that** the flavor is menthol.

## Patentansprüche

1. Verfahren zum Herstellen eines blattförmigen, Aromastoff-enthaltenden Materials für eine Zigarette, **dadurch gekennzeichnet, dass** das Verfahren die Schritte umfasst:
(i) Mischen eines Polysaccharids mit Wasser und Erhitzen der Mischung bei einer Temperatur von 60 bis 90°C, um eine wässrige Lösung des Polysaccharids herzustellen;
(ii) Zugeben eines Aromastoffs und eines Emulgators zur wässrigen Lösung des Polysaccharids und Kneten und Emulgieren der Lösung, um eine emulgierte Aufschlämmung zu erhalten; und
(iii) Gießen der emulgierten Aufschlämmung auf ein Substrat und Trocknen derselben, um eine Blattform zu erhalten,
wobei das Polysaccharid ein Ein-Komponenten-System von Tamarindengummi, Psyllium-Samengummi, oder Konjak-Glucomannan ist, oder ein Zusammensetzungssystem von zwei oder mehr kombinierten Bestandteilen, die ausgewählt sind aus der Gruppe, bestehend aus Tamarindengummi, Konjak-Glucomannan, Kassiengummi und Psyllium-Samengummi.

2. Verfahren nach Anspruch 1, **dadurch gekennzeichnet, dass** das Verfahren weiter den Schritt des Zerkleinern des erhaltenen blattförmigen, Aromastoffenthaltenden Materials für eine Zigarette umfasst.

3. Verfahren nach Anspruch 1 oder 2, **dadurch gekennzeichnet, dass** der Aromastoff Menthol ist.

## Revendications

1. Procédé de production d'un matériau contenant un arôme en forme de feuille pour cigarette, **caractérisé en ce que** le procédé comprend les étapes :
(i) de mélange d'un polysaccharide avec de l'eau et de chauffage du mélange à une température de 60 à 90°C pour préparer une solution aqueuse du polysaccharide ;
(ii) d'addition d'un arôme et d'un émulsionnant à la solution aqueuse du polysaccharide et de malaxage et d'émulsification de la solution pour obtenir une suspension émulsionnée ; et
(iii) de coulée de la suspension émulsionnée sur un substrat et de séchage de celle-ci pour obtenir une forme de feuille,
dans lequel le polysaccharide est un système monoconstituant de gomme de tamarin, de gomme de graine de psyllium ou de glucomannane de konjak, ou un système de composition de deux ou plusieurs constituants combinés choisis dans le groupe constitué de gomme de tamarin, de glucomannane de konjak, de gomme de cassia et de gomme de graine de psyllium.

2. Procédé selon la revendication 1, **caractérisé en ce que** le procédé comprend de plus l'étape de déchiquetage du matériau contenant un arôme en forme de feuille pour cigarette obtenu.

3. Procédé selon la revendication 1 ou 2, **caractérisé en ce que** l'arôme est le menthol.
